

# United States Patent Office

2,994,648  
Patented Aug. 1, 1961

## 1

2,994,648

### NICKEL PLATING ADDITIVES

Arthur H. Du Rose, Euclid, Ohio, assignor to The Harshaw Chemical Company, Cleveland, Ohio, a corporation of Ohio

No Drawing. Filed Apr. 22, 1960, Ser. No. 23,900

10 Claims. (Cl. 204—49)

This invention relates to the electrodeposition of nickel and more specifically to a process of electrodepositing nickel, and to a solution for use in a process for electrodepositing nickel. The invention has to do with the discovery of cooperating brightening agents suitable for use in aqueous acid nickel plating solutions where the solution contains a nickel electrolyte selected from nickel sulfate and nickel chloride and mixtures thereof.

According to the discovery, excellent bright, ductile and smooth deposits of nickel can be produced over a wide cathode current density range by electrolyzing an aqueous acid solution of a nickel electrolyte of the class consisting of nickel sulfate, nickel chloride and mixtures of nickel sulfate and nickel chloride if the solution also contains an effective amount of each of two cooperating addition agents.

One of the cooperating addition agents has an internal sulfur atom in the organic molecule and is characterized by a solubility in the plating solution of at least 0.0005 gram per liter and the following characteristic structure:



wherein X is a member selected from the group consisting of



and n and m are integers from 1 to 4, and A is a member

## 2

selected from the group consisting of H, CN—, CN—(CH<sub>2</sub>)<sub>p</sub>—O—, where p is an integer from 1 to 4, CN—(CH<sub>2</sub>)<sub>p</sub>—X—, where p is an integer from 1 to 4 and where X is a member selected from the group consisting of



10 and B is a member selected from the group consisting of —CN, —CN—(CH<sub>2</sub>)<sub>p</sub>—O, where p is an integer from 1 to 4 and CN—(CH<sub>2</sub>)<sub>p</sub>—X, where p is an integer from 1 to 4 and X is a member selected from the group consisting of



The preferred types are the symmetrical forms



where X is a member selected from the group consisting of



and n is an integer from 1 to 4, which may be called sulfonylalkylene nitriles and sulfinylalkylene nitriles.

30 The addition agents falling within this classification will hereafter be referred to as "brighteners." Typical brighteners according to the invention are indicated in Table I. The optimum range of each brightener which should be dissolved in the plating solution is also indicated in Table I in grams of brightener per liter of plating solution. They may be used in the plating solution in concentration from 0.0005 to 0.10 gram per liter.

Table I

|                                                                                      | Optimum Range, Grams per Liter |
|--------------------------------------------------------------------------------------|--------------------------------|
| (1) Bis(B-cyanoethyl) sulfone                                                        | 0.005-0.03                     |
|  |                                |
| (2) 1,4-Bis(B-cyanoethylsulfonyl)butane                                              | 0.005-0.03                     |
|  |                                |
| (3) Bis(B-cyanoethyl)sulfoxide                                                       | 0.005-0.03                     |
|  |                                |
| (4) B-cyanoethyl propyl sulfoxide                                                    | 0.008-0.05                     |
|  |                                |
| (5) B-cyanoethyl B-cyanoethoxyethyl sulfone                                          | 0.008-0.05                     |
|  |                                |
| (6) Bis(B-cyanoethoxyethyl)sulfone                                                   | 0.008-0.05                     |
|  |                                |

The second addition agent, which cooperates with the brightener in electrolytic, acid, nickel plating solutions

carrier is dissolved in the plating solution in amounts from about 2 to about 5 grams per liter.

Table II  
AROMATIC SULFONAMIDES

|                                                              |                                                    |
|--------------------------------------------------------------|----------------------------------------------------|
| benzene monosulfonamide.....                                 | $C_6H_5SO_2NH_2$                                   |
| saccharine, sodium salt.....                                 | $C_6H_5SO_2CONNa_2$                                |
| p-toluenesulfonamide.....                                    | $CH_3C_6H_4SO_2NH_2$                               |
| trichlorodibenzene sulfonamide.....                          | $Cl_3C_6H_2SO_2NHSO_2C_6H_4Cl$                     |
| di-B-naphthalenesulfonamide.....                             | $C_{10}H_7SO_2NHSO_2C_6H_7$                        |
| 4-carboxy dibenzene sulfonamide.....                         | $C_6H_5SO_2NHSO_2C_6H_4COOH$                       |
| N, N'-bis (phenylsulfonyl)-4, 4'-diphenyl disulfonamide..... | $C_6H_5SO_2NHSO_2C_6H_4C_6H_4SO_2NHSO_2C_6H_5$     |
| p, p'-oxy-bis (dibenzene sulfonamide).....                   | $C_6H_5SO_2NHSO_2C_6H_4OC_6H_4SO_2NHSO_2C_6H_5$    |
| p, p'-methylene-bis-(dibenzene sulfonamide).....             | $C_6H_5SO_2NHSO_2C_6H_4CH_2C_6H_4SO_2NHSO_2C_6H_5$ |

## AROMATIC SULFONATES

|                                      |                       |
|--------------------------------------|-----------------------|
| benzene monosulfonic acid.....       | $C_6H_5SO_3H$         |
| benzene disulfonic acid.....         | $C_6H_4(SO_3H)_2$     |
| nickel naphthalene disulfonate.....  | $C_{10}H_8(SO_3)_2Ni$ |
| cobalt naphthalene disulfonate.....  | $(C_6H_5SO_3)_2Co$    |
| nickel benzene monosulfonate.....    | $(C_6H_5SO_3)_2Ni$    |
| dichlorobenzene disulfonic acid..... | $Cl_2C_6H_4(SO_3H)_2$ |
| toluene sulfonic acid.....           | $CH_3C_6H_4SO_3H$     |
| diphenyl sulfonic acid.....          | $C_6H_5C_6H_4SO_3H$   |
| thiophene sulfonic acid.....         | $C_4H_9S.CO_3H$       |
| diphenyl sulfone.....                | $C_6H_5SO_2C_6H_5$    |
| naphthalene trisulfonic acid.....    | $C_{10}H_4(SO_3H)_3$  |

## UNSATURATED ALIPHATIC SULFONAMIDES AND SULFONIC ACIDS

|                             |                       |
|-----------------------------|-----------------------|
| Sodium vinyl sulfonate..... | $H_2C=CHSO_3Na$       |
| sodium allyl sulfonate..... | $H_2C=CHCH_2SO_3Na$   |
| vinyl sulfonamide.....      | $H_2C=CHSO_2NH_2$     |
| allyl sulfonamide.....      | $H_2C=CHCH_2SO_2NH_2$ |

falls into the category of organic sulfonamides, sulfimides, and sulfonates. The organic sulfonates, sulfimides and sulfonamides, according to the invention, comprise aromatic and unsaturated aliphatic sulfonates, sulfonamides, and sulfimides. Within the scope of the expression "aromatic and unsaturated aliphatic sulfonates, sulfonamides and sulfimides" are included the acids and their salts such as the sodium, potassium, nickel, cobalt, and iron salts thereof. Specifically, the class includes aryl and unsaturated alkyl sulfonates, sulfimides and sulfonamides, and the foregoing salts thereof wherein the number of carbon atoms in any aryl nucleus is from 6 to 10 and in any unsaturated alkyl group is from 1 to 10, and substitution products of the foregoing wherein the substituents are chosen from the class of alkyl groups having 1 to 4 carbon atoms, chlorine, CHO and phenyl. The organic sulfonamides, sulfimides, and sulfonates are frequently referred to as "carriers" or "control agents" in the art of nickel plating, and accordingly, are sometimes so-called herein. These carriers produce a degree of brightness without a cooperating brightener. Nevertheless, they do not produce sufficient brightness when utilized as the sole brightening additive in acid nickel plating solutions to be considered as producing a full, bright plate. The carriers or control agents constituting this second class of addition agents have a minimum solubility in the plating solution (for example, in a solution consisting of 240 grams of  $NiSO_4 \cdot 6H_2O$ , 37.5 grams of  $NiCl_2 \cdot 6H_2O$ , 37.5 grams of  $H_3BO_3$ , and water to make a liter) to the extent of at least 0.05 gram per liter.

Typical compounds illustrating the aryl and unsaturated alkyl sulfonamides, sulfimides and sulfonates are set forth in Table II. With respect to the aromatic sulfonic acids and sulfonamides and sulfimides various substituents in the ring structure are evident in the formulas indicated.

The brightening addition agent should be dissolved in the aqueous plating bath in an amount ranging from 0.0005 to 0.10 gram per liter. Optimum results are usually secured if the concentration of the brighteners dissolved in the aqueous plating bath ranges from about 0.005 to about 0.05 gram of brightener per liter of solution. The amount of carrier dissolved in the acid nickel plating solution ranges from .05 gram per liter to 20 grams per liter, best results being obtained when the

35 The constituents of the plating bath, according to the preferred practice of the invention, are (1) water, (2) nickel sulfate, nickel chloride, or a mixture of nickel sulfate and nickel chloride, (3) the brightener, (4) a sulfonate, a sulfonamide, a sulfimide, or one or more sulfonates, sulfonamides, sulfimides or mixtures thereof of the type previously indicated, and (5) and a wetting agent (optional). An additional ingredient of the solution which is desirable is a buffering agent such as boric acid, formic acid, or the like.

40 It will be noted that in reference to the major constituent of the nickel plating solution, the solutions are similar to the well known "all chloride," "all sulfate," and "sulfate-chloride" or "Watts" type acid nickel plating solutions. The essential novel feature of the invention is the use of an acid nickel plating solution having one or more nickel electrolytes selected from nickel sulfate and nickel chloride and additionally containing cooperating brightening agents, one of which is at least one 45 carrier selected from the group consisting of unsaturated aliphatic sulfonamides, unsaturated aliphatic sulfimides, unsaturated aliphatic sulfonates, aromatic sulfonamides, aromatic sulfimides and aromatic sulfonates, and the other of which is a small amount of a brightener of the 50 type heretofore indicated.

55 The basic solutions in connection with which the bright ductile nickel deposits are realized when containing the cooperating addition agents dissolved therein are as follows:

60 **ALL SULFATE**

|                                                    |                                                |
|----------------------------------------------------|------------------------------------------------|
| $NiSO_4 \cdot 7H_2O$ .....                         | 100 to 400 grams, preferably 200 to 300 grams. |
| Boric acid.....                                    | 0 to 60 grams, preferably 10 to 40 grams.      |
| 65 Wetting agent (e.g. sodium lauryl sulfate)..... | 0 to 0.5 grams, preferably 0.05 to 0.2 gram.   |
| $H_2O$ to make 1000 cc.                            |                                                |

70 **ALL CHLORIDE**

|                                                    |                                               |
|----------------------------------------------------|-----------------------------------------------|
| $NiCl_2 \cdot 6H_2O$ .....                         | 50 to 250 grams, preferably 100 to 200 grams. |
| Boric acid.....                                    | 0 to 60 grams, preferably 10 to 40 grams.     |
| 75 Wetting agent (e.g. sodium lauryl sulfate)..... | 0 to 0.5 grams, preferably 0.05 to 0.2 gram.  |
| $H_2O$ to make 1000 cc.                            |                                               |

## SULFATE-CHLORIDE WATTS TYPE

|                                                                                |                                                                                   |
|--------------------------------------------------------------------------------|-----------------------------------------------------------------------------------|
| NiSO <sub>4</sub> ·7H <sub>2</sub> O                                           | 100 to 400 grams, preferably 200 to 300 grams.                                    |
| NiCl <sub>2</sub> ·6H <sub>2</sub> O                                           | 10 to 60 grams, preferably 25 to 40 grams.                                        |
| Boric acid                                                                     | 0 to 50 grams, preferably 15 to 40 grams.                                         |
| Wetting agent (e.g. sodium sulfate derivative of 7-ethyl-2-methyl-undecanol-4) | 0 to 0.5 gram, preferably 0.025 to 0.2 gram.<br>H <sub>2</sub> O to make 1000 cc. |

The plating solutions above identified may be operated under conditions of pH, temperature, and cathode current density which are customarily employed therewith. When the cooperating brightening agents of the invention are dissolved in the plating solutions in the amount previously indicated, bright, ductile deposits will be obtained upon electrolysis of the solution. Typical operating conditions for the basic solutions are as follows:

|                                                  | All Sulfate | All Chloride | Watts   |
|--------------------------------------------------|-------------|--------------|---------|
| pH                                               | 3-4.5       | 2.4-4.5      | 3-4.5   |
| Temperature, ° F                                 | 120-160     | 100-150      | 110-155 |
| Cathode Current Density (amp./ft. <sup>2</sup> ) | 20-40       | 60-200       | 30-70   |

In the preparation of the plating solution according to the invention, I add to each of the foregoing basic solutions a suitable quantity of the brightener and also one or more of the unsaturated aliphatic, or aromatic sulfonamides, sulfimides, and sulfonates. The plating solution, for the best results, contains an antipitting agent although the deposits may be suitable for some purposes without eliminating pitting. Sodium lauryl sulfate or other wetting agents such as the sodium sulfate derivative of 7-ethyl-2-

methyl-undecanol-4 and the dihexyl ester of sodium sulfosuccinic acid may be used as an antipitting agent, although its use is not essential and other wetting agents or mixtures of wetting agents may be used to control the pitting. For some purposes pitting may be tolerated and sometimes very little pitting occurs.

Specific examples of electroplating solutions containing different cooperating brighteners and carriers are illustrated in Table III. The operating conditions for obtaining bright ductile nickel deposits are also set forth in the table. In each case a bright nickel deposit of from .05 to about 1 mil thick or thicker, may be secured by electrolyzing the electroplating solution between an anode and a buffed brass cathode. Similar results may be secured on other types of cathodes conventionally employed in acid nickel plating processes utilizing solutions of the type indicated herein.

According to one form of the invention, the addition of coumarin, or certain of its derivatives to the plating solution in amounts from .03 to .25 gram per liter and preferably about .1 gram per liter, materially aids in securing a smooth nickel deposit. Substituted coumarin derivatives where the substituents are alkyl or acyl groups not exceeding 4 carbon atoms, halogen, hydroxy or carboxy groups may be employed. Typical examples of substituted coumarins are 4-methyl coumarin, 6-chloro coumarin, 3-acetyl coumarin, coumarin-3-carboxylic acid, 4,8-dimethyl coumarin, 7-hydroxy coumarin, 6-carboxy coumarin, 3-chloro coumarin, 3-bromo coumarin, and 3-methyl coumarin. Thus, coumarin or its said derivatives may be dissolved in the nickel plating solutions containing the co-operating brightening agents and found to exert a leveling or smoothing action such that bright, ductile, nickel deposits of excellent smoothness are obtained.

Table III

|                                                  |       |      |        |      |        |       |      |      |      |       |       |
|--------------------------------------------------|-------|------|--------|------|--------|-------|------|------|------|-------|-------|
| Nickel Sulfate, g./l.                            | 300   | 300  | 300    | 300  | 300    | 300   | 300  | 300  | 300  | 300   | 10    |
| Nickel Fluoborate, g./l.                         |       |      |        |      |        |       |      |      |      |       |       |
| Nickel Chloride, g./l.                           | 38    | 38   | 38     | 38   | 38     | 38    | 38   | 38   | 38   | 38    | 38    |
| Boric Acid, g./l.                                | 38    | 38   | 38     | 38   | 38     | 38    | 38   | 38   | 38   | 38    | 38    |
| Allyl Sulfonic Acid, g./l.                       |       |      |        |      |        |       |      |      |      |       |       |
| Dibenzene Sulfonamide (Nickel salt), g./l.       | 3     |      |        |      |        |       |      |      |      |       |       |
| Naphthalene Disulfonate, g./l.                   |       | 2    | 2      |      | 2      |       |      |      | 2    |       |       |
| Allyl Sulfonamide, g./l.                         |       |      |        |      |        |       |      |      |      |       |       |
| Bi-dibenzenesulfonamide, g./l.                   |       |      | 3      | 3    | 3      | 3     | 3    | 3    | 3    | 3     |       |
| Dibenzenesulfonamide ether, g./l.                |       | 3    | 3      |      | 3      |       |      |      |      |       | 3     |
| Saccharin (sodium salt), g./l.                   | 1     |      |        |      |        |       |      |      |      |       | 2     |
| Toluene sulfonamide, g./l.                       |       |      |        |      |        |       |      |      |      |       |       |
| Bis(B-cyanoethyl)sulfone, g./l.                  | 0.01  |      | 0.0075 | 0.01 |        | 0.005 |      |      | 0.01 |       |       |
| 1,4-Bis(B-cyanoethylsulfonyl)butane, g./l.       |       |      |        |      |        |       |      |      |      |       |       |
| Bis(B-cyanoethyl) sulfoxide, g./l.               |       |      |        |      |        |       |      |      |      |       |       |
| B-cyanoethyl propyl sulfoxide, g./l.             | 0.010 |      |        |      |        |       |      |      | 0.01 |       |       |
| B-cyanoethyl B-cyanoethoxyethyl sulfone, g./l.   |       |      |        |      |        |       |      |      |      |       |       |
| Bis(B-cyanoethoxyethyl) sulfone, g./l.           |       |      |        |      | 0.015  |       |      |      |      | 0.015 |       |
| Coumarin, g./l.                                  |       | 0.1  |        |      |        | 0.05  |      |      |      |       | 0.015 |
| Cathode Current Density (amp./ft. <sup>2</sup> ) | 50    | 50   | 100    | 50   | 50     | 100   | 50   | 50   | 50   | 50    | 100   |
| Temperature, ° F                                 | 140   | 140  | 160    | 140  | 140    | 150   | 140  | 140  | 140  | 140   | 140   |
| Agitation <sup>1</sup>                           | C.R.  | C.R. | Air    | C.R. | C.R.   | Air   | C.R. | C.R. | C.R. | C.R.  | C.R.  |
| Nickel Sulfate, g./l.                            | 10    | 300  | 300    | 300  | 300    | 300   | 300  | 300  | 300  | 300   | 300   |
| Nickel Fluoborate, g./l.                         |       |      |        |      |        |       |      |      |      |       |       |
| Nickel Chloride, g./l.                           | 300   | 38   | 38     | 38   | 38     | 38    | 38   | 38   | 38   | 38    | 38    |
| Boric Acid, g./l.                                | 38    | 38   | 38     | 38   | 38     | 38    | 38   | 38   | 38   | 38    | 38    |
| Allyl Sulfonic Acid, g./l.                       | 1     |      | 1      |      |        |       |      |      |      |       |       |
| Dibenzene Sulfonamide (Nickel salt), g./l.       |       |      |        |      |        |       |      |      |      |       |       |
| Naphthalene Disulfonate, g./l.                   |       |      |        |      |        |       |      |      | 1    |       | 1     |
| Allyl Sulfonamide, g./l.                         |       |      |        |      |        |       |      |      |      |       |       |
| Bi-dibenzenesulfonamide, g./l.                   |       |      |        | 1    | 2      |       | 3    | 3    | 3    |       | 3     |
| Dibenzenesulfonamide ether, g./l.                |       | 3    |        |      |        | 3     | 3    |      |      |       |       |
| Saccharin (sodium salt), g./l.                   | 2     |      |        |      |        |       |      |      |      |       |       |
| Toluene sulfonamide, g./l.                       |       |      |        |      |        |       |      |      |      |       |       |
| Bis(B-cyanoethyl)sulfone, g./l.                  | 0.005 |      | 0.01   |      | 0.01   |       |      |      |      |       | 0.01  |
| Bis(B-cyanoethyl) sulfoxide, g./l.               |       |      |        |      | 0.0075 |       |      |      |      |       |       |
| B-cyanoethyl propyl sulfoxide, g./l.             |       |      |        |      |        | 0.015 |      |      | 0.01 |       |       |
| B-cyanoethyl B-cyanoethoxyethyl sulfone, g./l.   |       |      | 0.02   |      |        |       | 0.02 |      |      | 0.015 |       |
| Bis(B-cyanoethoxyethyl) sulfone, g./l.           |       |      |        |      |        |       | 0.02 |      | 0.05 | 0.05  |       |
| Coumarin, g./l.                                  |       |      |        |      |        |       |      |      | 0.05 | 0.05  |       |
| Cathode Current Density (amp./ft. <sup>2</sup> ) | 150   | 50   | 50     | 50   | 50     | 50    | 50   | 50   | 50   | 50    | 50    |
| Temperature, ° F                                 | 140   | 140  | 140    | 140  | 140    | 140   | 140  | 140  | 140  | 140   | 140   |
| Agitation <sup>1</sup>                           | Air   | C.R. | C.R.   | Air  | C.R.   | C.R.  | C.R. | C.R. | C.R. | C.R.  | C.R.  |

<sup>1</sup> C.R. = cathode rod.

What I claim is:

1. A nickel electroplating bath comprising an aqueous solution of nickel electrolyte selected from the group consisting of nickel sulfate, nickel chloride, and mixtures thereof, said solution also containing cooperating brightening addition agents, one of said brightening addition agents being at least one organic compound selected from the group consisting of aromatic and unsaturated aliphatic sulfonates, sulfonamides, and sulfimides, and the second of said brightening addition agents being a compound of the formula



wherein X is a member selected from the group consisting of



and n and m are integers from 1 to 4, and A is a member selected from the group consisting of H, CN—, CN—(CH<sub>2</sub>)<sub>p</sub>—O—, where p is an integer from 1 to 4, CN—(CH<sub>2</sub>)<sub>p</sub>—X—, where p is an integer from 1 to 4 and where X is a member selected from the group consisting of



and B is a member selected from the group consisting of —CN, —CN—(CH<sub>2</sub>)<sub>p</sub>—O—, where p is an integer from 1 to 4, and CN—(CH<sub>2</sub>)<sub>p</sub>—X— where p is an integer from 1 to 4 and X is a member selected from the group consisting of



the first said brightening addition agent being present in said solution to the extent of from .05 to 20 grams per liter and the second said brightening addition agent being present in said solution to the extent of from 0.0005 to 0.10 gram per liter.

2. A nickel electroplating bath comprising an aqueous solution of a nickel electrolyte selected from the group consisting of nickel sulfate, nickel chloride, and mixtures thereof, said solution also containing cooperating brightening addition agents, one of said brightening addition agents being at least one organic compound selected from the group consisting of aromatic and unsaturated aliphatic sulfonates, sulfonamides and sulfimides and the second of said agents being a compound of the formula



where X is a member selected from the group consisting of



and n is an integer from 1 to 4, the first said brightening addition agent being present in said solution to the extent of from .05 to 20 grams per liter and the second said brightening addition agent being present in said solution to the extent of from 0.0005 to 0.10 gram per liter.

3. A nickel electroplating bath comprising an aqueous solution of a nickel electrolyte selected from the group consisting of nickel sulfate, nickel chloride, and mixtures thereof, said solution also containing cooperating brightening addition agents, one of said brightening addition agents being at least one organic compound selected from the group consisting of aromatic and unsaturated aliphatic sulfonates, sulfonamides and sulfimides and the second

of said brightening addition agents being a compound of the formula



wherein n is an integer from 1 to 4, the first said brightening addition agent being present in said solution to the extent of from .05 to 20 grams per liter and the second 10 said brightening addition agent being present in said solution to the extent of from 0.0005 to 0.10 gram per liter.

4. A nickel electroplating bath comprising an aqueous solution of a nickel electrolyte selected from the group consisting of nickel sulfate, nickel chloride, and mixtures thereof, said solution also containing cooperating brightening addition agents, one of said brightening addition agents being at least one organic compound selected from the group consisting of aromatic and unsaturated aliphatic sulfonates, sulfonamides and sulfimides and the second 15 of said brightening addition agents being a compound of the formula



wherein n is an integer from 1 to 4, the first said brightening addition agent being present in said solution to the extent of from .05 to 20 grams per liter and the second 20 said brightening addition agent being present in said solution to the extent of from 0.0005 to 0.10 gram per liter.

5. An acid nickel electroplating solution comprising in addition to water, nickel sulfate equivalent to from 100 to 400 grams per liter of  $\text{NiSO}_4 \cdot 7\text{H}_2\text{O}$ , nickel chloride equivalent to from 10 to 60 grams per liter of  $\text{NiCl}_2 \cdot 6\text{H}_2\text{O}$ , a buffering agent and cooperating, brightening addition agents, one of said brightening addition agents being a compound selected from the group consisting of aromatic and unsaturated aliphatic sulfonates, sulfonamides and sulfimides and the second of said 35 brightening addition agents being Bis(B-cyanoethyl) sulfone, the first said brightening addition agent being present in said solution to the extent of from 0.05 to 20 grams per liter and the second said brightening addition agent being present in said solution to the extent of from 0.005 to 0.03 gram per liter.

6. An acid nickel electroplating solution comprising in addition to water, nickel sulfate equivalent to from 100 to 400 grams per liter of  $\text{NiSO}_4 \cdot 7\text{H}_2\text{O}$ , nickel chloride equivalent to from 10 to 60 grams per liter of  $\text{NiCl}_2 \cdot 6\text{H}_2\text{O}$ , a buffering agent and cooperating, brightening addition agents, one of said brightening addition agents being a compound selected from the group consisting of aromatic and unsaturated aliphatic sulfonates, sulfonamides and sulfimides and the second of said 50 brightening addition agents being a 1,4-Bis(B-cyanoethylsulfonyl) butane, the first said brightening addition agent being present in said solution to the extent of from 0.05 to 20 grams per liter and the second said brightening addition agent being present in said solution to the extent of from 0.005 to 0.03 gram per liter.

7. An acid nickel electroplating solution comprising in addition to water, nickel sulfate equivalent to from 100 to 400 grams per liter of  $\text{NiSO}_4 \cdot 7\text{H}_2\text{O}$ , nickel chloride equivalent to from 10 to 60 grams per liter of  $\text{NiCl}_2 \cdot 6\text{H}_2\text{O}$ , a buffering agent and cooperating, brightening addition agents, one of said brightening addition agents being a compound selected from the group consisting of aromatic and unsaturated aliphatic sulfonates, sulfonamides and sulfimides and the second of said 55 brightening addition agents being a Bis(B-cyanoethylsulfoxide, the first said brightening addition agent being present in said solution to the extent of from 0.05 to 20 grams per liter and the second said brightening addition agent being present in said solution to the extent of from 0.0005 to 0.006 gram per liter.

8. An acid nickel electroplating solution comprising in addition to water, nickel sulfate equivalent to from 100 to 400 grams per liter of  $\text{NiSO}_4 \cdot 7\text{H}_2\text{O}$ , nickel chloride equivalent to from 10 to 60 grams per liter of  $\text{NiCl}_2 \cdot 6\text{H}_2\text{O}$ , a buffering agent and cooperating, brightening addition agents, one of said brightening addition agents being a compound selected from the group consisting of aromatic and unsaturated aliphatic sulfonates, sulfonamides and sulfimides and the second of said brightening addition agents being a B-cyanoethyl propyl sulfoxide, the first said brightening addition agent being present in said solution to the extent of from 0.05 to 20 grams per liter and the second said brightening addition agent being present in said solution to the extent of from 0.0005 to 0.006 gram per liter.

9. An acid nickel electroplating solution comprising in addition to water, nickel sulfate equivalent to from 100 to 400 grams per liter of  $\text{NiSO}_4 \cdot 7\text{H}_2\text{O}$ , nickel chloride equivalent to from 10 to 60 grams per liter of  $\text{NiCl}_2 \cdot 6\text{H}_2\text{O}$ , a buffering agent and cooperating, brightening addition agents, one of said brightening addition agents being a compound selected from the group consisting of aromatic and unsaturated aliphatic sulfonates, sulfonamides and sulfimides and the second of said brightening addition agents being a B-cyanoethyl B-cyanoethoxyethyl sulfone, the first said brightening addition

agent being present in said solution to the extent of from 0.05 to 20 grams per liter and the second said brightening addition agent being present in said solution to the extent of from 0.0005 to 0.006 gram per liter.

8. 10. An acid nickel electroplating solution comprising in addition to water, nickel sulfate equivalent to from 100 to 400 grams per liter of  $\text{NiSO}_4 \cdot 7\text{H}_2\text{O}$ , nickel chloride equivalent to from 10 to 60 grams per liter of  $\text{NiCl}_2 \cdot 6\text{H}_2\text{O}$ , a buffering agent and cooperating, brightening addition agents, one of said brightening addition agents being a compound selected from the group consisting of aromatic and unsaturated aliphatic sulfonates, sulfonamides and sulfimides and the second of said brightening addition agents being a Bis(B-cyanoethoxyethyl) sulfone, the first said brightening addition agent being present in said solution to the extent of from 0.05 to 20 grams per liter and the second said brightening addition agent being present in said solution to the extent of from 0.0005 to 0.006 gram per liter.

20

**References Cited in the file of this patent**

**UNITED STATES PATENTS**

- |              |               |       |               |
|--------------|---------------|-------|---------------|
| 2,467,580    | Brown         | ----- | Apr. 19, 1949 |
| 25 2,882,208 | Becking et al | ----- | Apr. 14, 1959 |